



US005139692A

**United States Patent [19]**

Powell et al.

[11] Patent Number: **5,139,692**[45] Date of Patent: **Aug. 18, 1992****[54] ELECTRORHEOLOGICAL COMPOSITIONS INCLUDING AN AMINE-TERMINATED POLYESTER STERIC STABILIZER****[75] Inventors:** Bob R. Powell, Birmingham; Raymond L. Bloink, Swartz Creek, both of Mich.**[73] Assignee:** General Motors Corporation, Detroit, Mich.**[21] Appl. No.:** 702,990**[22] Filed:** May 20, 1991**[51] Int. Cl.<sup>5</sup>** C10M 171/00; C10M 169/04; C09K 3/00**[52] U.S. Cl.** 252/77; 252/75; 252/78.3; 252/572**[58] Field of Search** 252/75, 77, 78.3, 74, 252/572**[56] References Cited****U.S. PATENT DOCUMENTS**

|           |         |                 |             |
|-----------|---------|-----------------|-------------|
| 2,417,850 | 3/1947  | Winslow         | 175/320     |
| 3,839,252 | 10/1974 | Bosso et al.    | 260/29.2 EP |
| 4,645,614 | 2/1987  | Goossens et al. | 252/75      |
| 4,687,589 | 8/1987  | Block et al.    | 252/73      |
| 4,744,914 | 5/1988  | Filisko et al.  | 252/74      |
| 4,772,407 | 9/1988  | Carlson         | 252/74      |
| 4,879,056 | 11/1989 | Filisko et al.  | 252/74      |
| 4,927,464 | 5/1990  | Cowie           | 106/436     |

**FOREIGN PATENT DOCUMENTS**

|            |         |                    |
|------------|---------|--------------------|
| 0219323    | 4/1987  | European Pat. Off. |
| 0311984    | 4/1989  | European Pat. Off. |
| WO82/04442 | 12/1982 | PCT Int'l Appl.    |
| 1570234    | 6/1980  | United Kingdom     |

**OTHER PUBLICATIONS**

Matsepuro, "Structure Formation in an Electric Field and the Composition of Electrorheological Suspensions", translated from Elektroreol. Issled. Pril., Minsk, pp. 27-51, 1981.

Bridges et al., "Hyper-Dispersants-Applications in Air-Drying Paints", Chemical Abstracts 99(10), 72229y, 1983.

Jakubauskas, "Use of A-B Block Polymers as Dispersants for Non-Aqueous Coating Systems", Journal of

Coatings Technology, vol. 58, No. 736, May 1988, pp. 71-82.

Dispersion + Solsperse Hyperdispersants, Vendor's Brochure.

Material Safety Data Sheets #001125 #1531 and #1135, ICI Americas Inc., Wilmington, De. 19897.

Block et al., "Electro-Rheology", J. Phys. D: Appl. Phys., 21(12), 1661-77, 1988.

Hong et al., "High Na<sup>+</sup>-Ion Conductivity in Na<sub>5</sub>YSi<sub>4</sub>O<sub>12</sub>", Mat. Res. Bull., vol. 13, pp. 757-761, 1978. Pergamon Press, Inc. Printed in the U.S.

Clearfield et al., "New Crystalline Phases of Zirconium Phosphate Processing Ion-Exchange Properties", J. Inorg. Nucl. Chem. 1968, vol. 30, pp. 2249-2258. Pergamon Press. Printed in Great Britain.

Hong, "Crystal Structures and Crystal Chemistry in System Na<sub>1+x</sub>Zr<sub>2</sub>Si<sub>x</sub>P<sub>3-x</sub>O<sub>12</sub>", Mat. Res. Bull., vol. 11, pp. 173-182, 1976. Pergamon Press, Inc. Printed in the U.S.

Maazaz et al., "Sur Une Nouvelle Famille De Conducteurs Cationiques A Structure Feuilletee De Formule K<sub>x</sub>(L<sub>x</sub>/2Sn<sub>1-x</sub>/2)O<sub>2</sub>(L=Mg, Ca, Zn, x<1)", Mat. Res. Bull., vol. 14, pp. 193-199, 1979. Printed in the USA. 0025-5408/79/020193-782.00/0 Copyright (c) Pergamon Press Ltd.

Goodenough et al., "Fast Na<sup>+</sup>-Ion Transport in Skeleton Structures", Mat. Res. Bull., vol. 11, pp. 203-220, 1976. Pergamon Press, Inc. Printed in the U.S.

A selective portion of a book entitled "Introduction to Ceramics", pp. 859-863.

(List continued on next page.)

**Primary Examiner**—Paul Lieberman**Assistant Examiner**—Christine A. Skane**Attorney, Agent, or Firm**—Cary W. Brooks**[57]****ABSTRACT**

Disclosed are electrorheological fluids having zeolite particles and a nonconducting or dielectric fluid. The liquid phase includes an amine-terminated polyester to improve stability of the fluid.

**4 Claims, 1 Drawing Sheet**

## OTHER PUBLICATIONS

- Alberti et al., "All Solid State Hydrogen Sensors Based on Pellicular  $\alpha$ -Zirconium Phosphate as a Protonic Conductor", *Solid State Ionics*, vol. 35, No. 1, 2 Jul.-/Aug. 1989, pp. 153-156.
- Shannon et al., "Ionic Conductivity in  $\text{Na}_5\text{YSiO}_4$ -2-Type Silicates", *Inorganic Chemistry*, vol. 17, No. 4, 1978, pp. 958-964.
- Miller et al., "A Pre pilot Process for the Fabrication of Polycrystalline  $\beta$ "-Alumina Electrolyte Tubing", *Ceramic Bulletin*, vol. 58, No. 5 (1979), pp. 522-526.
- Scott et al., "ER Fluid Devices Near Commercial Stage", *International Viewpoints*, vol. 93, No. 11, pp. 75-79.
- Hooper et al., "Ionic Conductivity of Pure and Doped  $\text{Na}_3\text{PO}_4$ ", *Journal of Solid State Chemistry* 24, 265-275 (1978).
- West, "Ionic Conductivity of Oxides Based on  $\text{Li}_4\text{SiO}_4$ ", *Journal of Applied Electrochemistry* 3 (1973), pp. 327-335.
- Hu et al., "Ionic Conductivity of Lithium Phosphate-Doped Lithium Orthosilicate", *Mat. Res. Bull.*, vol. 11, pp. 1227-1230, 1976. Pergamon Press, Inc. Printed in the U.S.
- Hu et al., "Ionic Conductivity of Lithium Orthosilicate-Lithium Phosphate Solid Solutions", *J. Electrochem. Soc.:Solid-State Science and Technology*, vol. 124, No. 8, Aug. 1977, pp. 1240-1242.
- Delmas et al., "Ionic Conductivity in Sheet Oxides", Copyright 1979 by Elsevier North Holland, Inc. Vashishta, Mundy, Shenoy, eds. *Fast Ion Transport in Solids*, pp. 451-454.
- Delmas, "Sur De Nouveaux Conducteurs Ioniques A Structure Lamellaire", *Mat. Res. Bull.*, vol. 11, pp. 1081-1086, 1976. Pergamon Press, Inc. Printed in U.S.



FIG. 1

**ELECTRORHEOLOGICAL COMPOSITIONS  
INCLUDING AN AMINE-TERMINATED  
POLYESTER STERIC STABILIZER**

**FIELD OF THE INVENTION**

The present invention relates to fluid compositions which demonstrate significant changes in their flow properties in the presence of an electric field.

**BACKGROUND OF THE INVENTION**

Electrorheology is a phenomenon in which the rheology of a fluid is modified by the imposition of an electric field. Fluids which exhibit significant changes in their properties of flow in the presence of an electric field have been known for several decades. The phenomenon of electrorheology was reported by W. M. Winslow, U.S. Pat. No. 2,417,850, in 1947. Winslow demonstrated that certain suspensions of solids in liquids show large, reversible electrorheological effects. In the absence of an electric field, electrorheological fluids generally exhibit Newtonian behavior. That is, the applied force per unit area, known as shear stress, is directly proportional to the shear rate, i.e., change in velocity per unit thickness. When an electric field is applied, a yield stress appears and no shearing takes place until the shear stress exceeds a yield value which generally rises with increasing electric field strength. This phenomenon can appear as an increase in viscosity of up to several, and often many orders of magnitude. The response time to electric fields is on the order of milliseconds. This rapid response, characteristic of electrorheological fluids, makes them attractive to use as elements in mechanical devices.

A complete understanding of the mechanisms through which electrorheological fluids exhibit their particular behavior has eluded workers in the art. Many have speculated on the mechanisms giving rise to the behavior characteristics of electrorheological fluids.

A first theory is that the applied electric field restricts the freedom of particles to rotate, thus changing their bulk behavior.

A second theory ascribes the change in properties to the filament-like aggregates which form along the lines of the applied electric field. The theory proposes that this "induced fibrillation" results from small, lateral migrations of particles to regions of high field intensity between gaps of incomplete chains of particles, followed by mutual attraction of these particles. Criticism of a simple fibrillation theory has been made on the grounds that the electrorheological effect is much too rapid for such extensive structure formation to occur; workers in the art have observed a time scale for fibrillation of approximately 20 seconds, which is vastly in excess of the time scale for rheological response of electrorheological fluids. On the other hand, response times for fibrillation on the order of milliseconds have been observed.

A third theory refers to an "electric double layer" in which the effect is explained by hypothesizing that the application of an electric field causes ionic species adsorbed upon the discrete phase particles to move, relative to the particles, in the direction along the field toward the electrode having a charge opposite that of the mobile ions in the adsorbed layer. The resulting charge separation and polarization could lead to "dipole" interactions and fibrillation.

Yet another theory proposes that the electric field drives water to the surface of discrete phase particles through a process of electro-osmosis. The resulting water film on the particles then acts as a glue which holds particles together. If correct, then a possible sequence of events in fibrillation would be: ionic migration, subsequent electro-osmosis of moisture to one pole of the particle (presumably the cationic region) and bridging via this surface supply of water. However, the advent of anhydrous electrorheological fluids means that water-bridging is not an essential mechanism and may indeed not be operative at all.

Despite the numerous theories and speculations, it is generally agreed that the initial step in development of electrorheological behavior involves polarization under the influence of an electric field. This then induces some form of interaction between particles or between particles and the impressed electric or shear fields which results in the rheological manifestations of the effect. See Carlson, U.S. Pat. No. 4,772,407; and Block et al "Electro-Rheology", IEEE Symposium, London, 1985. Despite this one generally accepted mechanism, the development of suitable electrorheological fluids and methods of improving the same remains largely unpredictable.

The potential usefulness of electrorheological fluids in automotive applications, such as vibration damping, shock absorbers, or torque transfer, stems from their ability to increase, by orders of magnitude, their viscosity upon application of an electric field. This increase can be achieved with very fast (on the order of milliseconds) response times and with minimal power requirements.

Although ER-fluids have been formulated and investigated since the early 1940's, basic limitations have prevented their utilization in practical devices. The most restrictive requirements are (1) that the suspensions be stable over time; i.e., that the solid particles either remain suspended in the liquid or be readily redispersed if sedimentation occurs and (2) service and durability of the suspensions can be achieved outside the temperature range of 0°-100° C. This latter requirement is particularly restrictive in that most fluid compositions require water as an ER "activator" so that in completely nonaqueous systems the ER-effect is entirely absent or so small that it is not effectively useful.

An object of this invention is to formulate a stable, substantially water-free, or nonaqueous ER-fluid with improved properties.

**SUMMARY OF THE INVENTION**

This invention generally includes electrorheological fluids having a solid phase, an electrically nonconducting or dielectric fluid, and an amine-terminated polyester dispersant.

These and other objects, features and advantages of this invention will be apparent from the following detailed description, appended drawings and claims.

**BRIEF DESCRIPTION OF THE DRAWINGS**

FIG. 1 is a graphic illustration of the viscosity of an electrorheological fluid according to the present invention both in the presence and absence of an electric field.

## DETAILED DESCRIPTION OF THE INVENTION

The stability of an electrorheological fluid may be improved by adding a dispersant. When the liquid phase is a mineral oil, a preferred dispersant is an amine-terminated polyester. Preferably the amine-terminated polyester includes SOLSPERSE 17000 TM, 9000 TM, 3000 TM and preferably SOLSPERSE 17000 TM available from ICI Americas. The use of the amine-terminated polyester alters the interaction between the solid phase particles. The additive promotes weak bonding between the particles so as to flocculate (gel or agglomerate) the suspension. The flocculation prevents irreversible settling of the particles and does not interfere with ER behavior because the weak bonds between the particles are easily broken by slight agitation. The use of the additive does not inhibit the ER response of the fluid when AC fields are used. The use of the additive does not significantly alter the electric conductivity of the fluid. Preferably, the dispersant may be present in an amount ranging from about 0.6 to about 4.0, and most preferably 4 percent by weight of the total ER fluid. For optimizing the stability of the fluid, the additive-to-zeolite weight ratio is the critical parameter since it is then independent of the zeolite concentration in the electrorheological fluid. For example, 4 percent by weight of the additive in an electrorheological fluid containing 15 volume percent zeolite corresponds to an additive-to-zeolite weight ratio of 0.133. The amount of dispersant, and thus the additive-to-zeolite weight ratio, should be sufficient to keep the solid particles either suspended in the liquid or be readily redispersed if sedimentation occurs as described above.

It is believed that the amine-terminated polyester anchors to the particle on one end and extends out into the liquid phase on the other end. This structural arrangement keeps particles from settling out of suspension, presumably because the particles bond weakly to one another thereby creating a weak skeletal structure. It is possible that too high a concentration of additive would be disadvantageous because even weak interactions would be prevented and the particles would settle into a dense and not easily redispersed sediment. However, the outwardly extending amine-terminated polyester chains may inhibit the mobility of the particle in the liquid phase. Nevertheless, it was surprisingly found that the amine-terminated polyester dispersant did not inhibit the ER response of fluids containing the dispersant in an AC electric field. However, the dispersant did inhibit the ER response in a DC electric field. It was also surprisingly found that repeated cycling from field-off to field-on conditions did not affect the ability of the dispersant to adhere to the particles and keep them readily dispersible in the liquid phase.

The solid phase of an electrorheological fluid according to the present invention may be prepared from any zeolite material. The term "zeolite" as used in this invention means the family of hydrated silicates having an open framework and is intersected by wide channels in which cations and water molecules are located. A preferred material may be prepared from the zeolite phase having the formula  $M_{(x/n)}[(AlO_2)_x(SiO_2)_y].zH_2O$ , where M is a metal cation or mixtures of metal cations of average valence charge n; x and y are integers and z is a variable and most favorably comprises the zeolite phase  $Na_{12}[(AlO_2)_{12}(SiO_2)_{12}].zH_2O$ . Particularly preferred materials for the solid phase are commercially

available from Union Carbide, under the trade names Type 4A Zeolite TM and Type 4A Molecular Sieve TM.

Preferably, the materials of the solid phase are in the form of particles such as spheres, cubes, whiskers and platelets. Preferably, the particles are equiaxed. The particles have an effective length or diameter ranging from about 0.1 to about 75 micrometers. The particles may be present in the fluid in an amount ranging from about 5 to about 50, and preferably about 15 to about 30 percent by volume of the composition.

Preferably, the material of the solid phase is dried at a temperature ranging from about 200° C. to about 600° C., preferably 400° C. to about 600° C. and most preferably 600° C., which is sufficient to remove any residual water on the solid phase but not alter the structure of the solid. The particles are referred to as being substantially free of water. The term "substantially free of water" means less than 0.5 percent by weight water adhering (i.e., absorbed or adsorbed) to the particles. Preferably, the amount of water adhering to the particles is less than that required for the water to be an "activator" of electrorheological response. That is, the amount of water adhering to the particles of the solid phase is not sufficient to create water bridges between particles under the influence of an electric field. The drying of the particles is carried out under low vacuum at a constant pressure. Preferably the drying is at a pressure ranging from about 300 to about 50 mTorr, preferably 200 to about 50 mTorr and most preferably at 50 mTorr. The resultant, dry particles are then dispersed in a liquid phase. Suitable liquid phase materials include any nonconductive or dielectric substance that exists in a liquid state under the conditions which an electrorheological fluid made using it would be employed. Preferably the liquid is a mineral oil. Other suitable liquid phase materials are disclosed in Block et al, "Electro-Rheology", IEEE Symposium, London, 1985, which is hereby incorporated by reference. A suitable mineral oil is commercially available from CITCO under the trade name Sentry 39 TM.

Electrorheological fluids were prepared as described above wherein the solid phase consisted of a material having the composition  $Na_{12}[(AlO_2)_{12}(SiO_2)_{12}].zH_2O$  and the liquid phase consisted of mineral oil and varying amounts of dispersant. As can be seen in FIG. 1, in the presence of an electric field the fluids exhibited a dramatic increase in viscosity compared to the fluid in the absence of electric field.

The various embodiments may be combined and varied in a manner within the ordinary skill of persons in the art to practice the invention and to achieve various results as desired.

Where particular aspects of the present invention is defined herein in terms of ranges, it is intended that the invention includes the entire range so defined, and any sub-range or multiple sub-ranges within the broad range. By way of example, where the invention is described as comprising one to about 100 percent by weight component A, it is intended to convey the invention as including about five to about 25 percent by weight component A, and about 50 to about 75 percent by weight component A. Likewise, where the present invention has been described herein as including A<sub>1-100</sub>-B<sub>1-50</sub>, it is intended to convey the invention as A<sub>1-60</sub>-B<sub>1-20</sub>, A<sub>60-100</sub>B<sub>25-50</sub> and A<sub>43</sub>B<sub>37</sub>.

The embodiments of the invention in which an exclusive property or privilege is claimed are defined as follows:

1. A method of producing an electrorheological response and a composition comprising:

providing a composition comprising conductive or semiconductive particles, present in an amount ranging from about 5 to about 50 percent by volume of said composition, a mineral oil, and an amine-terminated polyester steric stabilizer, said stabilizer being present in an amount ranging from about 0.6 to about 4 weight percent of said composition; and

applying an electric field to said composition to increase the viscosity of said composition.

2. A method as set forth in claim 1 wherein said solid phase comprises zeolite particles.

3. A method as set forth in claim 1 wherein said solid phase comprises a material prepared from a zeolite phase having the formula:



10

where M is a metal cation or mixtures of metal cations of average valence charge n; x and y are integers and z is a variable.

4. A method as set forth in claim 1 wherein said solid phase comprises a material prepared from the zeolite phase  $Na_{12}[(AlO_2)(SiO_2)_{12}].zH_2O$ .

\* \* \* \* \*

20

25

30

35

40

45

50

55

60

65